

## UNITED STATES PATENT OFFICE

2,353,587

INHIBITING FOAMING OF VISCOSUS  
PETROLEUM OILCarroll N. Rill, Jackson Heights, N. Y., assignor  
to Socony-Vacuum Oil Company, Incorporated,  
New York, N. Y., a corporation of New YorkNo Drawing. Application February 19, 1941,  
Serial No. 379,645

## 3 Claims. (Cl. 252—317)

This invention has to do with the use of viscous oils such as gear oils, transmission oils, hydraulic oils and the like where the oil is used in an enclosed system and is subjected to vigorous agitation in use.

An oil of the type contemplated herein may be employed as a lubricant or it may serve the dual purpose of lubrication and power transmission, but irrespective of the purpose accomplished by these oils they have in common the feature of operating in enclosed systems, in most cases completely filled with oil, where any increase in volume due to foaming results in leakage and loss of product. Such a loss results in loss of lubrication and, in case of hydraulic oils, in decreased efficiency of power transmission.

Heretofore it has been the practice to produce gear oils and similar products which normally have a low or slight tendency to foam under conditions of use, by the selection of suitable petroleum stocks and refining methods to yield such a product, the final properties being largely dependent upon the selection of raw materials.

It is the primary object of this invention to provide a method to prevent the foaming of an oil of the class described which is normally susceptible to foaming under the conditions of vigorous agitation encountered in use by adding to the oil a minor proportion of an ingredient which will act as an anti-foaming agent. This invention also contemplates as a composition of matter, the viscous oil composition containing the anti-foaming agent.

My invention is predicated upon the discovery that three organic thiophosphates, namely tricapryl monothiophosphate, triamyl-monothiophosphate and tri 2-ethyl-hexyl monothiophosphate are highly effective as anti-foaming agents while many other organic compounds of phosphorus including some other thiophosphates had little or no effect in that regard.

This unexpected property of the three thiophosphates contemplated herein is demonstrated by the test results set forth in Table I below where the foam retarding properties of these three thiophosphates are compared with the results obtained under similar test conditions with other organic compounds of phosphorus including other thiophosphates. The test employed in obtaining the data in Table I was an accelerated service test simulating the actual working conditions of transmission and hydraulic oils. In this test a 50 cc. sample of oil is placed in a 1.5 in. I. D. graduate and violently agitated with a hair-

pin stirrer driven at 1750 R. P. M. for 20 minutes, after which the stirrer is removed from the oil and the total volume of oil is observed and recorded. The volume percent of foam formed from 50 cc. of the original oil is a measure of the foaming tendency of the oil or oil blend. Readings were also made of the time required for the foam to subside so that a bull's eye of clear oil could be seen through the foam. Two different oil stocks were used in the test. Oil A in the table below was a mineral gear oil having a Saybolt viscosity of 85 seconds at 210° F. and oil B was mineral gear oil having a Saybolt viscosity of 250 seconds at 210° F.

Table

| Oil | Compound added                       | Per cent | Temp. of test<br>°F. | Per cent<br>foam after<br>agitation | Time for<br>appearance<br>of clear<br>oil surface |
|-----|--------------------------------------|----------|----------------------|-------------------------------------|---------------------------------------------------|
|     |                                      |          |                      |                                     | Minutes                                           |
| A   | None                                 |          | 100                  | 70                                  | 45                                                |
| A   | Tricapryl monothiophosphate.         | 1        | 100                  | None                                |                                                   |
| A   | Triamyl monothiophosphate.           | 1        | 100                  | 16                                  | 42                                                |
| A   | Triphenyl tetrathiophosphate.        | 1        | 100                  | 100                                 | 150                                               |
| A   | Triphenyl trithiophosphate.          | 1        | 100                  | 98                                  | 150                                               |
| A   | Tri oleyl monothiophosphate.         | 1        | 100                  | 98                                  | 150                                               |
| A   | Tri beta phenyl ethyl thiophosphate. | 1        | 100                  | 90                                  | 150                                               |
| A   | Dioleyl dithiophosphate.             | 1        | 100                  | 100                                 | 150                                               |
| B   | None                                 |          | 100                  | 108                                 | 239                                               |
| B   | Tricapryl monothiophosphate.         | 1        | 100                  | None                                |                                                   |
| B   | Triamyl monothiophosphate.           | 1        | 100                  | None                                |                                                   |
| B   | Tri 2-ethyl-hexyl monothiophosphate. | 1        | 100                  | 20                                  | 127                                               |
| B   | None                                 |          | 78                   | 36                                  | 360                                               |
| B   | Tricapryl monothiophosphate.         | 1        | 78                   | 2                                   |                                                   |
| B   | Trioleyl monothiophosphate.          | 1        | 78                   | 70                                  | 360                                               |
| B   | Tri beta phenyl ethyl thiophosphate. | 1        | 78                   | 88                                  | 300                                               |

From the foregoing test results it will be seen that thiophosphates from the group consisting of tricapryl monothiophosphate, triamyl monothiophosphate and tri 2-ethyl-hexyl monothiophosphate are effective to materially reduce, and in some instances to entirely eliminate, the foaming tendency of the oil while the other phosphates tested actually increased the foaming tendency.

The monothiophosphates contemplated herein as anti-foaming agents may be used in the oil in amounts ranging from about 0.1 percent to about 5.0 percent.

I claim:

1. In the method of utilizing a viscous petroleum oil in a system wherein the oil is subjected to vigorous agitation and normally tends to develop a substantial quantity of foam, the step of inhibiting the foaming of the oil by incorporating therein a minor proportion, from about 0.1 percent to about 5.0 percent, of a thiophosphate selected from the group consisting of tri-capryl monothiophosphate, and tri-2-ethyl-hexyl-monothiophosphate.
2. In the method of utilizing a viscous petroleum oil in a system wherein the oil is subjected to vigorous agitation and normally tends to de-

velop a substantial quantity of foam, the step of inhibiting the foaming of the oil by incorporating therein a minor proportion, from about 0.1 percent to about 5.0 percent of tri-capryl-monothiophosphate.

- 5 3. In the method of utilizing a viscous petroleum oil in a system wherein the oil is subjected to vigorous agitation and normally tends to develop a substantial quantity of foam, the step of inhibiting the foaming of the oil by incorporating therein a minor proportion from about 0.1 percent to about 5.0 percent of tri-2-ethyl-hexyl monothiophosphate.

CARROLL N. RILL.